



US005801325A

**United States Patent** [19]

Willer et al.

[11] Patent Number: 5,801,325

[45] Date of Patent: Sep. 1, 1998

[54] **HIGH PERFORMANCE LARGE LAUNCH VEHICLE SOLID PROPELLANTS**

[75] Inventors: Rodney L. Willer, Newark, Del.; David K. McGrath, Elkton, Md.

[73] Assignee: Cordant Technologies Inc., Ogden, Utah

[21] Appl. No.: 561,774

[22] Filed: Aug. 2, 1990

[51] Int. Cl. 5 C06D 45/10

[52] U.S. Cl. 149/19.4; 149/19.6

[58] Field of Search 149/19.7, 19.6

[56] **References Cited****U.S. PATENT DOCUMENTS**

|           |         |                      |           |
|-----------|---------|----------------------|-----------|
| 3,004,840 | 10/1961 | Pruitt et al.        | 149/19.4  |
| 3,291,660 | 12/1966 | Oberth et al.        | 149/19.4  |
| 3,305,565 | 2/1967  | Mueller              | 260/348.6 |
| 3,531,534 | 9/1970  | Adolph               | 260/614   |
| 3,557,181 | 1/1971  | Lakritz et al.       | 260/453   |
| 3,756,874 | 9/1973  | Chang et al.         | 149/19.4  |
| 3,870,578 | 3/1975  | Nichols              | 149/19.4  |
| 4,158,583 | 6/1979  | Frosch               | 149/19.4  |
| 4,184,031 | 1/1980  | Graham et al.        | 149/19.4  |
| 4,393,199 | 7/1983  | Manser               | 528/408   |
| 4,483,978 | 11/1984 | Manser               | 149/19.4  |
| 4,511,742 | 4/1985  | Yu                   | 568/621   |
| 4,726,919 | 2/1988  | Kristofferson et al. | 149/19.4  |
| 4,799,980 | 1/1989  | Reed, Jr.            | 149/19.4  |
| 4,915,755 | 4/1990  | Kim                  | 149/19.4  |
| 4,952,254 | 8/1990  | Betts et al.         | 149/19.4  |
| 4,976,794 | 12/1990 | Biddle et al.        | 149/19.5  |

**OTHER PUBLICATIONS**

S.D. Morse, Polymerization and Modifications of Low Molecular Weight Polyethers, U. of Dayton Research Inst., Report No. UDR-TR-83-116, 40 pp, Oct. 1983.

R. Willer et al., Proceedings of the Jt. Int'l Symp. on Comp. of Plastics and other Mat'l's with Expl., Prop., Pyrotech and Processing of Expl., Prop. and Ingredients, 23-25 Oct. 1989, Virginia Beach, VA, pp. 258-269.

E. Colclough et al., Proceedings of the Jt. Int'l Symp. on Comp. of Plastics and other Mat'l's with Expl., Prop., Pyrotech and Processing of Expl., Prop. and Ingredients, 23-25 Oct. 1989, Virginia Beach, VA, pp. 235-240.

D. Debenham, Proceedings of the Jt. Int'l Symp. on Comp. of Plastics and other Mat'l's with Expl., Prop., Pyrotech and Processing of Expl., Prop. and Ingredients, 23-25 Oct. 1989, Virginia Beach, VA, pp. 119-129.

S. Penczek et al., Lecture at IUPAC 6th Int'l Symp. on "Cationic Polymerization & Related Processes", E.J. Goethals Ed., Academic Press, 1984, pp. 139-154.

K. Brzezinska et al., Makromol. Chem., Rapid Commun., 7, pp. 1-4, (1986).

S. Penczek et al., Makromol. Chem., Macromol. Symp., 3, pp. 203-217 (1986).

M. Bednarek et al., Makromol. Chem. Suppl., 15, pp. 49-60 (1989).

C. C. Gonzales et al., Makromol. Chem., 190, pp. 1217-1224 (1989).

Naval Ordnance Laboratory NAVWEPS Report 7409, A Survey of Nitro-Organic Compounds Related to Solid Propellant Systems (U), pp. 34-37, 61-64, 121, 129, 130, 132, 134, 137, 138, 143-146, Jun. 20, 1961.

U.S. Naval Ordnance, NAVORD Report 2028, Polyglycidyl Nitrate, Part 1, Preparation and Characterization of Glycidyl Nitrate, NOTS 685, 13 pages plus abstract, May 6, 1953.

U.S. Naval Ordnance, NAVORD Report 2028, Polyglycidyl Nitrate, Part 2, Preparation and Characterization of Polyglycidyl Nitrate, NOTS 686, 20 pages plus abstract, May 7, 1953.

Jet Propulsion Laboratory, Publication No. 93, High-Performance Polyglycidyl Nitrate-Polyurethane Propellants, 33 pages, Mar. 29, 1957.

Defense Technical Information Center (DTIC), Document No. AD 144756, 1957.

Defense Technical Information Center (DTIC), Document No. AD 139462, 1957.

ACS Symp. Series 286, Ring-Opening Polymerization Kinetics, Mechanism and Synthesis, Chapter 25, Cationic Ring-Opening Polymerization of Epichlorohydrin in the Presence of Ethylene Glycol, Y. Ohamoto, pp. 361-372, J.E. McGrath, editor, ACS 1985.

ACS Symp. Series 286, Ring-Opening Polymerization Kinetics, Mechanism and Synthesis, Chapter 20, Homopolymerization of Epoxides in the Presence of Fluorinated Carbon Acids, J. Robins et al, pp. 263-274, J.E. McGrath, editor, ACS 1985.

Translation of article by Y.I. Estrin et al, Vysokomol. soyed., A10: No. 11, Kinetics of Polymerization of Epichlorohydrin Glycidyl Nitrate Catalyzed by  $\text{BF}_3$ , pp. 2589-2599, 1968.

Translation of article by A.I. Kuzayev et al, Vysokomol. soyed., A11: No. 5, Polymerization Kinetics of Tetrahydrofuran Caused by  $\text{BF}_3\text{-THF}$  in the Presence of Glycidyl Nitrate in 1,2-Dichloroethane, pp. 989-994, 1969.

Translation of article by S.G. Entelis et al, Vysokomol. soyed., A13: No. 6, Regularities of Cationic Polymerization of Cyclic Ethers, pp. 1438-1446, 1971.

G.V. Korovina et al., J. Poly. Science: Part C, No. 16 pp. 3575-3579 (1968).

**Primary Examiner**—Edward A. Miller

**Attorney, Agent, or Firm**—Pillsbury, Madison & Sutro LLP; Cushman, Darby & Cushman Intellectual Property Group; Ronald L. Lyons

[57] **ABSTRACT**

A family of high performance, large launch vehicle, solid propellants based on polyglycidyl nitrate elastomer binders. A clean, large launch vehicle, solid propellant based on a polyglycidyl nitrate elastomer binder, ammonium nitrate oxidizer and aluminum or magnesium fuel optimizes at low solids levels and produces essentially no HCl or chloride ion in the exhaust.

**14 Claims, No Drawings**

## HIGH PERFORMANCE LARGE LAUNCH VEHICLE SOLID PROPELLANTS

### FIELD OF THE INVENTION

This invention relates to improved high performance, large launch vehicle solid propellants based on a polyglycidyl nitrate elastomer binder, ammonium nitrate oxidizer and aluminum or magnesium fuel and which optimize at low solids levels.

### BACKGROUND OF THE INVENTION

Solid high energy compositions, such as propellants, explosives, gasifiers, or the like, comprise solid particulates, such as fuel particulates and/or oxidizer particulates, dispersed and immobilized throughout a binder matrix comprising an elastomeric polymer.

Binders previously used in composite solid propellant formulations have generally been non-energetic polymers such as polycaprolactones, polyethyleneglycols or polybutadienes. Since about 1950 there has been a considerable need to develop energetic binders with satisfactory mechanical properties in order to provide safer binders at higher energy levels and to increase the energy level or specific impulse in a propellant formulation. For the most part only nitrocellulose has found usefulness as an energetic polymer binder. However, nitrocellulose suffers from undesirable mechanical properties. Alternatively, it has been proposed to employ conventional non-energetic polymer binders in combination with energetic plasticizers such as for example, nitroglycerine, butanetriol trinitrate, and trimethylolethane trinitrate. It has also been suggested that the energetic polymer nitrocellulose be employed with either non-energetic or energetic plasticizers in an attempt to improve mechanical properties. However, none of these proposals has led to fully acceptable energetic binder formulations.

Furthermore, there are many occasions when the use of plasticizers is undesirable or their use is not possible, such as when "clean" space motor/gas generator propellants or "clean" large launch vehicle propellants are required. The propellants used in the current generation of large solid rocket boosters, such as Delta, Titan and Space Shuttle, all employ ammonium perchlorate (AP) as the oxidizer and thus produce large amounts of HCl in their exhaust. The HCl is corrosive to metals sensors employed in, and around the rocket and is toxic to humans. Moreover, concern over the ozone layer's depletion has led to a desire to develop solid propellants for use in such booster rockets that would not produce HCl in their exhaust.

Several approaches have been taken to develop such large launch vehicle solid propellants which do not produce HCl in their exhaust or which produce reduced amounts of HCl in their exhaust. Most such approaches have used ammonium nitrate (AN) as the oxidizer or used a co-oxidizer along with AP, such as sodium nitrate, whose combustion products will scavenge (or neutralize) the HCl produced in the AP combustion. However, the lower oxidizing ability of AN and its melting has led to severe problems with the first, while complex combustion problems affect the second or scavenger approach. Moreover, the scavenger approach tends merely to neutralize HCl formed but does not get rid of chloride ions which are believed to add to the ozone layer depletion problem. Additionally, with the increasing number of Space Shuttle and other large vehicle launches the problem of HCl and chloride ion production can only be expected to become more severe.

Typical ammonium perchlorate-hydrocarbon large launch vehicle solid propellants optimize the specific impulse (Isp)

obtained at about 80%-90% wt. solids and have Isp's of approximately 250 to 260 lb-sec/lb at 1000 psi and sea-level optimal, expansion conditions.

Thus, there has been a continuing need for energetic polymers to be available for use in formulating solid high-energy compositions, such as propellants, explosives, gasifiers and the like. In this regard much recent work has centered on attempts to produce acceptable energetic polymers of glycidyl azide polymer and poly(oxytanes). A problem with elastomeric binders formed from poly(oxytanes) is their tendency to have mechanical characteristics less than that which would be desirable for a high-energy composition, particularly for a rocket motor propellant. It is especially difficult to provide poly(oxytane) binders having adequate stress capabilities. On the other hand glycidyl azide polymer is synthesized by first polymerizing epichlorohydrin to poly(epichlorohydrin) which is then converted to glycidyl azide polymer by reaction with sodium azide in dimethylsulfoxide. Beside the lack of a simple synthesis process, the production of glycidyl azide polymer requires relatively expensive reagents. Moreover, even after the polymer is synthesized it has been found that unplasticized glycidyl azide polymer-ammonium perchlorate solid propellants require about 78% solids to optimize Isp at about 254 sec.

Since the early 1950's poly(glycidyl nitrate), hereinafter referred to as PGN, has been known and recognized as a possible energetic prepolymer. The initial work on PGN was done by Thelan et al. at the Naval Ordnance Test Station (NOTS, now the Naval Weapons Center, NWC). They studied the polymerization of glycidyl nitrate by a variety of Lewis Acid catalysts with most of the work centering on the use of stannic chloride as a catalyst. No propellants were prepared by the NOTS workers and they noted that one drawback to their synthesis was the laborious purification procedure.

PGN AND PGN propellants were next examined at the Jet Propulsion Laboratory (JPL) by Ingman and Nichols and at Aerojet General Corporation by Shookhoff and Klotz. The JPL workers found that PGN made using boron trifluoride etherate was low in both functionality (i.e. <2) and molecular weight (MW=1500) and therefore polyurethane propellants made from this PGN had poor mechanical properties. Similar observations were made by the Aerojet workers. In summary, it has long been recognized that PGN may be an excellent energetic polymer but until now a method of synthesis could not be found that would produce nearly difunctional material with acceptable hydroxyl equivalent weights. Nor has it been possible to formulate acceptable unplasticized "clean" PGN large launch vehicle solid propellants having reduced levels of solids.

It is therefore desirable to provide a family of high energy, clean, large launch vehicle solid propellants and particularly such propellants which produce essentially no HCl or chloride ion in their exhaust. A further object of this invention is to provide such a family of high energy, clean, large launch vehicle solid propellants which employ ammonium nitrate as the oxidizer and do not require the use of ammonium perchlorate as the oxidizer. A still further object of this invention is to provide such high energy, clean, large launch vehicle solid propellants containing PGN elastomer binder, ammonium nitrate oxidizer and aluminum or magnesium as fuel. An even further object of this invention is to provide such high energy, clean, large launch vehicle solid propellants requiring reduced solids loading to obtain optimized performance as measured by the specific impulse of the propellants and yet producing essentially no HCl or chloride

ions in their exhaust. Yet another object of this invention is to provide such high energy, clean, large launch vehicle solid propellants which perform as well as or better than the current solid propellant employed for the Space Shuttle but which produces essentially no HCl or chloride ions in their exhaust.

### SUMMARY OF THE INVENTION

It has been discovered that high energy solid propellants which are clean, large launch vehicle solid propellants, not requiring the presence of a plasticizer, can be provided by utilizing a curable polyglycidyl nitrate (PGN) binder and a reduced amount of energetic ammonium nitrate oxidizer and aluminum or magnesium fuel solid particulate particles wherein the PGN employed is a PGN having a functionality of nearly 2.0 or more and a hydroxyl equivalent weight of about 1000-1700 or more. More preferably such high energy solid propellants which are clean, large launch vehicle solid propellants are provided by utilizing an isocyanate curable PGN binder having a functionality of nearly 2.0 or more, a hydroxyl equivalent weight of about 1200 to 1600 and wherein the PGN employed has less than about 2 to 5% by weight cyclic oligomer present in the PGN.

### DETAILED DESCRIPTION OF THE INVENTION

In U.S. Pat. No. 5,120,827 there is described a process for the production of PGN that produces nearly difunctional material with acceptable hydroxyl equivalent weights, particularly PGN having a functionality of nearly 2.0 or more, or essentially equivalent to the hydroxy functionality of the polyol initiator employed in the process, and a hydroxyl equivalent weight of about 1000-1700 or more, preferably about 1200 to 1600. Moreover, that Application provides a process for producing PGN that has present greatly reduced amounts of cyclic oligomer, that is about 2-5% by weight or less of said oligomer.

In said concurrently filed Application, the improved process for the production of PGN, in which cyclic oligomer formation is suppressed and PGN having a functionality substantially equal to the functionality of the polyol initiator and an acceptable hydroxyl equivalent weight is obtained, is provided by a process wherein a catalyst-initiator complex is formed and reacted with glycidyl nitrate (GN) and wherein the ratio of mols catalyst/mol hydroxyls in the initiator is <1:1, the glycidyl nitrate is added to the catalyst-initiator complex reaction mixture at a rate substantially equivalent to the rate at which it reacts with the complex such that no effective net amount of glycidyl nitrate monomer is built up, i.e. monomer is used up essentially as fast as it is added to the reaction mixture, and the reaction temperature is maintained within the range of from about 10°-25° C. Additionally, the process provides for the removal of any potential alkoxide groups, such as ethoxide groups, from the catalyst-initiator complex mixture when the catalyst employed in the process leads to the formation of such groups.

According to the process described in said concurrently filed Application glycidyl nitrate,



is polymerized to PGN,



initiator,

wherein n is an integer essentially equivalent to the hydroxy functionality of the initiator and x is an integer representing the repeating units, by forming a catalyst-initiator complex and reacting the complex with glycidyl nitrate and wherein the ratio of mols catalysts/mols hydroxyls in the initiator is <1:1, the glycidyl nitrate monomer is added to the catalyst-initiator complex reaction mixture at a rate in which the monomer is used up (reacted) essentially as fast as it is added, and the reaction temperature is maintained at a temperature within the range of from about 10° to 25° C.

The polymerization reaction is a cationic polymerization process conducted using a polyol initiator and an acid catalyst. The acid catalyst may be chosen from among those known in the art, including  $\text{BF}_3$ ,  $\text{HBF}_4$  and triethyloxonium hexafluorophosphate (TEOP). The Lewis acid catalyst forms a preinitiator complex with the polyol, for example, butanediol is known to form a complex with boron trifluoride ( $\text{BF}_3$ ).

The polyol initiator employed generally has the hydroxyl groups of the polyol unhindered. The polyol is preferably a diol. As examples of suitable diols there may be mentioned ethylene glycol, propylene glycol, 1,3-propanediol and 1,4-butanediol. Suitable triols include, but are not limited to glycerol, trimethylolpropane and 1,2,4-butanetriol. A suitable tetrol is, but is not limited to 2,2'-dihydroxymethyl-1,3-propanediol. The molecular weight of the polyol is relatively low, preferably less than 500, more preferably below 300 and most preferably below about 150.

The acid catalyst is used at a much lower level relative to hydroxyl groups of the polyol than is taught in the prior art. It was discovered that a much more controlled reaction occurs if the catalyst, such as a Lewis Acid, is used at a molar ratio relative to hydroxyl groups of the polyol of less than 1:1, preferably from about 0.4:1 to about 0.8:1. If a proton acid is used as the catalyst, the ratio of hydrogen ions released by the acid catalyst to the hydroxyl groups of the alcohol is also less than 1:1, preferably 0.4:1 to about 0.8:1. By using a substantially lower level of acid catalyst, incorporation of a greater percentage of the polyol molecules internally within polymer molecules is achieved, cyclic oligomer formation is suppressed to a level of about 2 to 5% or less, and lower polydispersity is achieved.

The cationic polymerization reaction may be carried out in a suitable organic solvent conducive to the cationic polymerization. If a solvent is employed, such suitable solvent is a non-protic, non-ether, inert solvent. Such solvents include, but are not limited to methylene chloride, chloroform, and 1,2-dichloroethane.

The polymerization reaction is conducted in a manner whereby the glycidyl nitrate monomer is added to the reaction mixture at a rate essentially equivalent to its rate of reaction, so that no effective net concentration of monomer is built up in the reaction mixture and the reaction temperature is maintained at a temperature within the range of from about 10° to 25° C., preferably from about 11° to 17° and most preferably about 13° to 15° C. It will be appreciated that the faster heat is taken away from the reactive mixture the faster glycidyl nitrate monomer can be added to the reaction mixture.

When the reaction of catalyst and initiator results in the formation of alkoxide groups in the catalyst-initiator

complex, such as for example, the presence of alkoxide group compounds in the reaction mixture formed by the reaction of boron trifluoride etherate and 1,4-butanediol, the resulting PGN products are low in functionality. Pre-reacting the polyol 1,4-butanediol and boron trifluoride etherate and then removing diethylether under vacuum produces a PGN product essentially free of alkoxide groups. If, however, the catalyst and initiator would not form products containing such alkoxide groups, such as when boron trifluoride gas is employed instead of boron trifluoride etherate, then prereaction of the catalyst and initiator and removal of potential alkoxide compounds is not necessary.

The hydroxyl equivalent weight of the PGN polymer produced according to this process will generally be from about 1000 to 1700 or more, preferably from about 1200 to about 1600 and the amount of cyclic oligomer produced will generally be about 2-5% by weight or less.

It has been discovered that the improved PGN produced according to the process of said concurrently filed Application permits the production of high energy solid propellants which are clean, large launch vehicle solid propellants not requiring the presence of a plasticizer. The high energy solid propellants of this invention require greatly reduced amounts of solid particulate materials in order to obtain optimized performance as measured by the specific impulse of the propellant. The solids content may be as low as about 60% by weight, and is preferably about 60-75% by weight. However, if desired, propellant formulations with higher solids contents of up to about 85% by weight can be formulated. The high energy solid propellants of this invention produce greatly reduced amounts of condensables and HCl, i.e. generally less than about 1.25% by weight condensables and less than about 7 mol % HCl, preferably about 0% of each. Furthermore, the lower solids levels permits better processability of the solid propellant formulations.

It is surprising that the PGN propellants of this invention provide optimized performance at reduced solid levels. With the plasticizer-free, reduced solids content solid propellants of this invention it is possible to obtain clean, large launch vehicle propellants with a specific impulse of about 250 to 260 or more pounds force-sec per pound mass at 1000 psi pressure and sea-level optimum expansion conditions.

Although a plasticizer is not required it will be recognized that it is possible to add suitable plasticizers to the solid propellants of this invention for applications wherein the presence of a plasticizer is not prohibited or is not undesirable. In such cases any suitable plasticizer may be employed and generally in an amount up to about a plasticizer to PGN weight ratio of about 2.5:1. As examples of suitable plasticizers which may be present in the high energy solid propellants there may be mentioned high-energy plasticizers such as nitroglycerine (NG), butanetriol trinitrate (BTTN), trimethylolethane trinitrate (TMETN) and triethylene glycol dinitrate (TEGDN).

The high energy, large launch vehicle solid propellants will generally comprise from about 60 or more wt. %, preferably 60-75 wt. %, particulate solids, including fuel material particulates and oxidizer particulates. Where it is unnecessary to have clean, reduced smoke solid propellants the particulate solids level in the propellants could, if desired, comprise also up to about 85% by weight or more. The fuel particulates employed in the large launch vehicle solid propellant formulations of this invention can be aluminum or magnesium or mixtures thereof with boron. Particulate oxidizer material employed is ammonium nitrate (AN) but can also include cyclotetramethylene tetranitramine (HMX), cyclotrimethylene trinitramine (RDX) and

other high energy nitramines such as CL-20 and the like and mixtures thereof. The high energy solid propellants may optionally include minor amounts of additional components known in the art, such as bonding agents, and burn rate modifiers such as diaminoglyoxime (DAG) or diaminofuran (DAF) and the like.

Cured PGN elastomers are formed by curing PGN with isocyanates having a functionality of at least two or more, such as for example, hexamethylene diisocyanate (HMDI), toluene diisocyanate (TDI), and polyfunctional isocyanates, such as for example, Desmodur N-100 available from the Mobay Chemical Co., a division of Farbenfabriken Bayer AG, and mixtures thereof.

The following is a typical example of a method for the preparation of poly(glycidyl nitrate) according to the aforementioned concurrently filed application, suitable for use in the high energy large launch vehicle solid propellants of this invention. A clean, dry, three neck r.b. flask is equipped with a vacuum adapter, rubber septum, magnetic stirring bar and a thermometer. The flask is charged with 29.7 g (0.33 mole) of dry 1,4-butanediol, cooled to 20° C. and 46.8 g (0.33 mole) of  $\text{BF}_3$  etherate is slowly added via a syringe while maintaining the temperature below 25° C. This mixture is stirred for 1 hr. at 25° C. then the ether is removed by pulling a partial vacuum for 1 hr. and a full vacuum for 16 hrs. Dry methylene chloride (175 ml) is added to the flask and the contents are transferred using a cannula to a clean dry 5 liter jacketed resin flask previously filled with 400 ml dry methylene chloride and cooled to 10° C. equipped with a mechanical stirrer, thermometer,  $\text{N}_2$  purge, and a peristaltic addition pump. An additional 25 ml of dry methylene chloride is used to insure quantitative transfer of the catalyst initiator complex. The temperature in the reactor is adjusted to  $13^\circ \pm 2^\circ$  C. and a solution of 1190 g (10 moles) of monomer grade glycidyl nitrate in 800 ml of dry methylene chloride is added at such a rate as to maintain a temperature of  $13^\circ \pm 2^\circ$  C. This typically takes 4.5 hours. The reaction is stirred for 0.5 hr. then quenched by the addition of 400 ml of a saturated sodium chloride solution. The brine solution is separated and the methylene chloride solution of PGN is washed three times with 500 ml of saturated sodium bicarbonate solution. The methylene chloride solution is dried over magnesium sulfate and the methylene chloride removed on a rotoevaporator at a pressure of <1 mm and a temperature of 40° C. (1 hr.) and 55° C. (2 hrs.) to give essentially a quantitative yield of poly(glycidyl nitrate) as a viscous light yellow liquid.

The invention is now illustrated in greater detail by way of the following illustrative examples. In all the following examples the PGN prepolymer employed in the binder of the solid propellants is one prepared according to the preceding illustrative preparation and having a molecular weight of about 2500 and a hydroxyl equivalent weight of about 1250. The binder contains about 0.47% at mononitroaniline (MNA) as a nitrate ester stabilizer and about 0.03% at triphenylbismuth (TPB) as a urethane cure catalyst. Theoretical specific impulse values are calculated according to the program described in Gordon, S. and McBride, B., "Computer Program for Calculation of Complex Chemical Equilibrium Composition, Rocket Performance, Incident and Reflected Shock and Chapman-Jouquet Detonations", NASA, SP-273 (1976).

Table I sets forth the theoretical specific impulses, densities and density Isp's for various high-energy, unplasticized large launch vehicle propellants at a 1000/14.7 psi pressure, namely for the present standard Space Shuttle propellant (PBAN), for various proposed large launch vehicle propellants of hydroxy terminated polybutadiene (HTPB) and glycidyl azide polymer (GAP) as well as for two PGN large launch vehicle propellant formulations of

this invention. The binder in the PGN propellants comprise the PGN prepolymer and HMDI curative isocyanate present in a 12/1 wt. ratio.

TABLE I

| Binder                              | Isp, Density and Density Isp for Large Launch Vehicle Propellants |       |                      |       |       |       |        |        |          |        |
|-------------------------------------|-------------------------------------------------------------------|-------|----------------------|-------|-------|-------|--------|--------|----------|--------|
|                                     | PBAN                                                              | HTPB  | HTPB                 | GAP   | PGN   | PGN   | PGN    | PGN    | PGN      | PGN    |
| Binder, % wt.                       | 14                                                                | 12    | 12                   | 30    | 30    | 30    | 30     | 30     | 30       | 25     |
| Oxidizer                            | AP                                                                | AP    | AP/NaNO <sub>3</sub> | AN    | AN    | AN    | AN/HMX | AN/HMX | AN/CL-20 | AN/RDX |
|                                     |                                                                   |       | (1:1)                |       |       |       | (3:1)  | (4:1)  | (3:1)    | (3:1)  |
| Oxidizer, % wt.                     | 70                                                                | 68    | 68                   | 50    | 50    | 50    | 48     | 50     | 48       | 53     |
| Al, % wt.                           | 16                                                                | 20    | 20                   | 20    | 20    | 22    | 22     | 20     | 22       | 22     |
| O/F ratio                           | 1.264                                                             | 1.188 | 1.206                | 1.037 | 1.456 | 1.340 | 1.177  | 1.301  | 1.178    | 1.177  |
| Isp, lb-sec/lb                      | 262.0                                                             | 265.3 | 246.0                | 259.7 | 259.6 | 260.7 | 264.0  | 262.4  | 263.9    | 264.0  |
| Density, lb/in <sup>3</sup>         | 0.063                                                             | 0.065 | 0.068                | 0.060 | 0.063 | 0.063 | 0.064  | 0.063  | 0.064    | 0.065  |
| Density Isp, lb-sec/in <sup>3</sup> | 16.63                                                             | 17.30 | 16.63                | 15.63 | 16.23 | 16.40 | 16.90  | 16.53  | 16.89    | 17.15  |

PBAN = polybutadiene acrylonitrile copolymer

GAP = glycidyl azide polymer

Table II sets forth theoretical Isp's and densities as well as the end of mix (EOM) viscosity and oxidizer/fuel (O/F) ratio for various high energy large launch vehicle PGN solid propellants employing magnesium as the fuel.

TABLE II

| Ex.<br>No. | Percent by weight |                 |                | EOM |                 | Isp, lb-sec/lb  |                   |              |
|------------|-------------------|-----------------|----------------|-----|-----------------|-----------------|-------------------|--------------|
|            | PGN               | AN<br>200 $\mu$ | AN<br>20 $\mu$ | MG  | Viscosity<br>kP | Density<br>g/cc | 1000-<br>14.7 psi | O/F<br>Ratio |
| 1          | 30                | 50              | —              | 20  | 96              | 1.618           | 254.0             | 3.37         |
| 2          | 60                | 20              | —              | 20  | 8               | 1.586           | 254.2             | 2.52         |
| 3          | 35                | 25              | 20             | 20  | 14              | 1.601           | 252.8             | 2.82         |
| 4          | 30                | 30              | 20             | 20  | 64              | 1.618           | 254.0             | 3.37         |
| 5          | 35                | 25              | 19             | 20  | 18              | 1.605           | 251.1             | 2.60         |

Ballistic properties for the formulations in Table II are set forth in Table III.

TABLE III

| Ex.<br>No. | Ballistic Properties            |          |                                 |          |
|------------|---------------------------------|----------|---------------------------------|----------|
|            | Burn Rate<br>1000 psi<br>in/sec | Exponent | Burn Rate<br>2000 psi<br>in/sec | Exponent |
| 1          | 0.29                            |          | 0.41                            | 0.75     |
| 2          | 0.29                            | .31      | 0.35                            | 0.73     |
| 3          |                                 |          | 0.37                            | 0.72     |
| 4          |                                 |          | 0.38                            | 0.75     |
| 5          |                                 |          | 0.37                            | 0.72     |

In Table IV there is set forth properties for two further PGN/AN/Al clean large launch vehicle solid propellants as well as for the current Space Shuttle propellant formulation as identified in Table I hereinbefore.

TABLE IV

| Example No.                 | 6    | 7    | Space<br>Shuttle |
|-----------------------------|------|------|------------------|
| Binder, %                   | 30   | 30   |                  |
| Curative N-100/HMDI (50:50) |      |      |                  |
| NCO/OH                      | 1.0  | 1.0  |                  |
| AN 200 $\mu$ , %            | 50.0 | 50.0 |                  |
| Al, %                       | 20.0 | 18.0 |                  |

TABLE IV-continued

| Example No.                   | 6      | 7      | Space<br>Shuttle |
|-------------------------------|--------|--------|------------------|
| B, %                          | —      | 2.0    |                  |
| Stress, lb/in <sup>2</sup>    | 1691   | 206    | 171              |
| Strain, in/in                 | 39     | 30     | 41               |
| Modulus, psi                  | 710    | 1100   | 855              |
| Burn rate, 2000 psi, in/sec   | 0.33   | 0.41   |                  |
| Burn rate, 1000 psi, in/sec   | 0.21   | 0.25   | 0.43             |
| Exponent                      | 0.72   | 0.62   | 0.35             |
| EOM viscosity, kP             | 14     | 12     | 18               |
| Density, g/cc                 | 1.731  | 1.707  | 1.744            |
| Isp, 1000-14.7 psi, lb-sec/lb | 259.26 | 257.90 | 262.0            |

Four hundred and fifty gram (450 g) batches of the solid propellants of Examples 6 and 7 were prepared in the following manners into a suitable mixing vessel, under vacuum, the PGN, MNA, aluminum and boron were added and mixed for about 15 minutes. To this mixture 50% by weight of the AN was added and mixed for a further 15 minutes after which the remaining AN was added and mixed for an additional 15 minute period. Then TPB in toluene was added and mixed for a further period of about 15 minutes followed by addition thereto of the N-100/HMDI mix which was subjected to a further mixing for a period of about 15 minutes. The propellant was allowed to cure for 3 days at about 135° F. This solid propellant possessed excellent mechanical and processing properties as shown by the data in Table IV. The inclusion of a small amount of boron increases the burn rate and reduces the burn rate pressure exponent.

Thus, this invention provides clean large launch vehicle solid propellants which are essentially equivalent to or better than current Space Shuttle solid propellant but which are "clean".

With the foregoing description of the invention, those skilled in the art will appreciate that modifications may be made to the invention without departing from the spirit thereof. Therefore, it is not intended that the scope of the invention be limited to the specific embodiments illustrated and described.

We claim:

1. A high energy, large launch vehicle, solid propellant having a theoretical specific impulse, at a pressure ratio of 1,000 psi to 14.7 psi, of at least about 250 lb-sec/lb and comprising an isocyanate cured polyglycidyl nitrate binder

and from about 60 to about 75% by weight high energy particulate solids comprising ammonium nitrate oxidizer particulates and fuel particulates selected from aluminum and magnesium and wherein the polyglycidyl nitrate is an isocyanate curable polyglycidyl nitrate polymer having a functionality of nearly 2.0 or more and a hydroxyl equivalent weight of from about 1000 to about 1700 and has less than about 2 to 5% by weight cyclic oligomer present in the polyglycidyl nitrate.

2. A high energy, large launch vehicle, solid propellant of claim 1 wherein the particulate solids comprise about 70% by weight.

3. A high energy, large launch vehicle, plasticizer-free, solid propellant comprising an isocyanate cured polyglycidyl nitrate binder and from about 60 to about 75% by weight high energy particulate solids comprising ammonium nitrate oxidizer and particulates and fuel particulates selected from aluminum and magnesium, wherein the polyglycidyl nitrate is an isocyanate curable polyglycidyl nitrate polymer having a functionality of nearly 2.0 or more and a hydroxyl equivalent weight of from about 1000 to about 1700 and has less than about 2 to 5% by weight cyclic oligomer present in the polyglycidyl nitrate and said solid propellant upon combustion producing less than about 1.25% weight condensables and less than about 7 mol % by weight HCl.

4. A high energy, large launch vehicle, plasticizer-free solid propellant of claim 3 wherein the particulate solids comprise about 70% by weight.

5. A high energy, large launch vehicle, plasticizer-free solid propellant of claim 3 wherein the fuel particulates also comprise aluminum.

6. A high energy, large launch vehicle, plasticizer-free solid propellant of claim 3 wherein the fuel particulates also comprise magnesium.

7. A high energy, large launch vehicle, plasticizer-free solid propellant of claim 5 wherein the particulates additionally comprise cyclotetramethylene tetranitramine, cyclotrimethylene trinitramine, CL-20, diaminoglyoxime and mixtures thereof.

8. A high energy, large launch vehicle, plasticizer-free solid propellant of claim 6 wherein the particulate solids

additionally comprise cyclotetramethylene tetranitramine, cyclotrimethylene trinitramine, CL-20, diaminoglyoxime and mixtures thereof.

9. A high energy, large launch vehicle, plasticizer-free solid propellant of claim 3 wherein the propellant includes additional components selected from bonding agent, burn rate modifier, nitrate ester stabilizer and urethane cure catalyst.

10. A high energy, large launch vehicle, plasticizer-free solid propellant of claim 5 wherein the propellant includes additional components selected from bonding agent, burn rate modifier, nitrate ester stabilizer and urethane cure catalyst.

11. A high energy, large launch vehicle, plasticizer-free solid propellant of claim 6 wherein the propellant includes additional components selected from bonding agent, burn rate modifier, nitrate ester stabilizer and urethane cure catalyst.

12. A high energy, large launch vehicle, solid propellant having a theoretical specific impulse, at a pressure ratio of 1,000 psi to 14.7 psi, of at least 250 lb-sec/lb and comprising about 15 to about 40% by weight of an isocyanate cured polyglycidyl nitrate binder and from about 60 to about 85% by weight of particulate solids and wherein the particulate solids comprise ammonium nitrate oxidizer particulates and fuel particulates selected from aluminum or magnesium and wherein the polyglycidyl nitrate is an isocyanate curable polyglycidyl nitrate polymer having a functionality of nearly 2.0 or more and a hydroxyl equivalent weight of from about 1000 to about 1700 and has less than about 2 to 5% by weight cyclic oligomer present in the polyglycidyl nitrate.

13. A high energy, large launch vehicle, solid propellant of claim 12 which is plasticizer free and upon combustion produces less than about 1.25% by weight condensables and less than about 7 mol % by weight HCl.

14. The propellant of claim 12 wherein the amount of binder is present in an amount of from about 25 to 40% by weight and particulate solids are present in an amount of from about 60 to 75% by weight.

\* \* \* \* \*